

Feb. 27, 1940.

O. DAHL ET AL

2,192,032

METHOD FOR IMPROVING THE MAGNETIC PROPERTIES OF FERROUS ALLOYS

Original Filed Feb. 15, 1936 2 Sheets-Sheet 1

Fig. 1.



Fig. 2.



Inventors:

Otto Dahl,  
Franz Pawlek,

by Harry E. Dunham  
Their Attorney.

Feb. 27, 1940.

O. DAHL ET AL

2,192,032

METHOD FOR IMPROVING THE MAGNETIC PROPERTIES OF FERROUS ALLOYS

Original Filed Feb. 15, 1936 2 Sheets-Sheet 2

Fig. 3.



Inventors:  
Otto Dahl,  
Franz Pawlek,  
by Harry E. Dunham  
Their Attorney.

## UNITED STATES PATENT OFFICE

2,192,032

## METHOD FOR IMPROVING THE MAGNETIC PROPERTIES OF FERROUS ALLOYS

Otto Dahl, Berlin-Friedenau, and Franz Pawlek, Berlin-Niederschönheide, Germany, assignors to General Electric Company, a corporation of New York

Original application February 15, 1936, Serial No. 64,138. Divided and this application October 26, 1938, Serial No. 237,156. In Germany March 11, 1935.

3 Claims. (Cl. 148—4)

This application is a division of our copending application, Serial No. 64,138, filed February 15, 1936, now Patent 2,145,712, January 31, 1939, and entitled Method for improving the magnetic properties of ferrous alloys.

In order to obtain a uniform rise of magnetization throughout a wide field-strength range, as well as a nearly complete saturation at low field strengths, it has been proposed to produce in magnetic materials, an ordered grain texture such as can be obtained by certain rolling and annealing processes. For instance, magnetic iron-nickel alloys can be cold-rolled, prior to the final annealing, with a reduction of thickness 10 amounting to more than 90%, preferably more than 95%, after which the material is annealed at temperatures above the recrystallization limit. As a result of this treatment, an ordered position of the crystallites is obtained in the plates 15 after the annealing, and this ordered position has an extraordinary favorable influence on the magnetic properties.

The present invention is an improvement of these methods and consists in subjecting the alloys during cooling, after the final annealing, to the influence of a magnetic field, in such a way that, depending upon whether the magnetization curves, as a function of the field strength, are to have a steeper or flatter shape, the alloys are 20 subjected either to the influence of a longitudinal or transverse magnetic field. The terms, longitudinal and transverse, here, imply respectively the direction of rolling or the direction at right angles to the direction of rolling. While 25 the influence of a magnetic field applied during the cooling is known, it has been found unexpectedly, that by applying simultaneously the methods for obtaining an ordered grain structure and the cooling under a magnetic field, the effect 30 on magnetic properties could be considerably increased, and that said properties could be given a degree of perfection such as has not been obtained so far.

In the attached drawings, we have indicated 35 graphically the results for three different alloy combinations. The curves denoted by "a" represent in each case, the results obtained with specimens which, for the purpose of an ordered grain structure, have been subjected, prior to the final 40 annealing, to a cold rolling resulting in a decrease in thickness exceeding 90%. On the other hand, the curves denoted by "b" represent the results obtained with specimens that had been subjected to a lesser amount of cold rolling such as had 45 been resorted to formerly. The indexes 1 to 3

indicate whether the alloy specimens were subjected to a magnetic field during the cooling and, if so, to what magnetic field. Specimens with index 1 were cooled without the application of a magnetic field; the specimens with index 2 were cooled with the simultaneous application of a longitudinal magnetic field, while specimens with index 3 were cooled with the simultaneous application of a transverse magnetic field.

Fig. 1 refers to a binary iron-nickel alloy with 10 40% nickel and 60% iron; Fig. 2 refers to a binary iron-nickel alloy having equal parts of iron and nickel, while Fig. 3 refers to an iron-nickel-cobalt alloy with 45% nickel, 30% iron and 25% cobalt. The alloy specimens were produced together and in exactly the same manner. All were obtained from a casting produced in a high frequency furnace from technically pure materials; they were then reduced to a thickness of 0.3 mm. by way of forging or hot or cold rolling with intermediate annealing above the recrystallization 15 temperature. The specimens of group b were subjected, during the last cold rolling to a decrease in thickness amounting to 80%, that is, a decrease in thickness which is close to the limit 20 of the conventional rolling process used in connection with such alloys. In contrast to this, the specimens of group a were, in order to attain a good grain structure, subjected to a last cold rolling, which resulted in a decrease in thickness 25 of 98.5%. Finally, all specimens were subjected to a last annealing at 1100° C. for two hours in a 30 hydrogen current.

The process, according to the invention, has 35 different qualitative results, depending on the different alloys. However, it has been found that by using simultaneously a high degree of cold rolling (for obtaining an ordered grain texture) and a longitudinal magnetic field during the cooling, there is always obtained a steeper magnetization 40 curve which extends linearly through a wider induction range. On the other hand, the simultaneous application of a high degree of cold rolling and of a transverse magnetic field during cooling, results always in a magnetizing curve 45 which is rectilinear through an unusually wide field-strength range. In particular, the magnetization characteristic of the alloy represented in Fig. 2, which consists of equal parts of iron and nickel, is steeper than that of the magnetization 50 curve of the alloy according to Fig. 1, which alloy has 40% of nickel and 60% of iron. Thus, if for certain reasons, a linear magnetization characteristic is desired through a field-strength 55 range which is as wide as possible, the alloy, ac-

cording to Fig. 1, should be given preference to the alloy according to Fig. 2. This condition will always obtain whenever the field strength cannot be reduced at will by the selection of a small 5 number of turns in a coil. However, if this reduction is possible, so that when dimensioning a coil, only the induction need be considered, the alloy, according to Fig. 2, should be given preference over the alloy of Fig. 1, for with the alloy, 10 according to Fig. 2, the same effect can be obtained with a smaller amount of material.

Fig. 3 shows that the application of the method, according to the invention, is not limited to binary iron-nickel alloys, but that it can be also successfully applied to the iron-nickel-cobalt alloys. The improvement of the steep rise of the characteristic by the simultaneous application of a high degree of cold rolling and a longitudinal magnetic field during the cooling is, here, not so 20 marked as was the case with the application of the longitudinal magnetic field in connection with the binary iron-nickel alloys, for the application of a magnetic field alone, permits obtaining a very steep curve. On the other hand, 25 the improvement of the linear rise through a wide field-strength range, by applying simultaneously a high degree of stretching and a transversal magnetic field, is here quite considerable; Fig. 3 shows that the uniform rise begins practically at the point of origin and that it continues until saturation sets in. The hysteresis 30 loop returns with the low remanence of a thousand gauss, nearly as linearly as it rises. Such an alloy is of major importance for communication engineering, for instance for Krarup lines, and also for transmitters, for a magnetic body 35 consisting of that particular alloy, operates practically without harmonics. For this reason, an alloy of that composition and treatment must be 40 primarily applied in all those cases which deal with circuits in which the harmonics have a disturbing effect, even at a slight amplitude. Such fields of application exist always in those cases when several signals are to be transmitted 45 through one and the same line by means of different carrier frequencies, for in these cases, the harmonics of one channel come within the transmitting range of the other channel and may thus entail a mutual interference of both channels.

50

The application of the object of the invention is not limited to the alloys which have been chosen by way of example. The entirely different composition of the alloys in Figs. 1 and 2 on the one hand, and in Fig. 3 on the other hand, 5 indicates plainly that the method according to the invention will permit a considerable influencing of the magnetic properties in nearly all ferromagnetic substances. Which one of the known alloys must be chosen for any particular purpose, can be determined from case to case by a simple test. The method is particularly advantageous in connection with all those alloys in which the application of the conventional annealing treatments alone, that is to say, primarily, 15 the application of a slower cooling will result in a rectilinear magnetization characteristic through a certain field strength range. These alloys are, on the one hand, the binary iron-nickel alloys with or without the addition of small quantities 20 of third substances (up to about 10%) and, on the other hand, the iron-nickel-cobalt alloys such as they have been described by Elmen.

What we claim as new and desire to secure by Letters Patent of the United States, is:

1. A method for improving the magnetic properties of alloys consisting of nickel and iron which comprises cold working the alloy to effect a reduction in thickness of more than 90%, annealing the alloy and during cooling subjecting it to 30 the influence of a transverse magnetic field.

2. A method for improving the magnetic properties of alloys consisting of iron and metal from the group nickel and cobalt which comprises cold working the alloy to effect a reduction in thickness of more than 90%, annealing said alloy and during cooling subjecting it to the influence of 35 a transverse magnetic field.

3. A method for improving the magnetic properties of alloys consisting of iron and metal from the group nickel and cobalt which comprises cold 40 rolling the alloy to effect a reduction in thickness of more than 90%, annealing the rolled metal and during cooling subjecting it to the influence of a magnetic field which is applied in 45 a direction transverse to the direction in which the metal was cold rolled.

OTTO DAHL.  
FRANZ PAWLEK.

50